

## UNITED STATES PATENT OFFICE.

ALBERT L. CLAPP, OF DANVERS, MASSACHUSETTS, ASSIGNOR TO BENNETT, INCORPORATED, OF BOSTON, MASSACHUSETTS, A CORPORATION OF MASSACHUSETTS.

## WATERPROOF PAPER AND PROCESS OF PRODUCING THE SAME.

No Drawing.

Application filed February 23, 1926. Serial No. 90,153.

This invention has relation to the production of waterproof paper, using aqueous dispersions comprising a high proportion of dispersed particles of various unsaponifiable or difficultly saponifiable waterproofing materials, such as mineral oils, waxes, bitumens, gums, resins, asphalts, and like materials as sizing agents. The present invention has for one of its objects to provide a process of sizing pulp prior to its formation into paper, in an efficacious and economical manner, with such aqueous dispersions.

Dispersions of thermoplastic waterproofing material may be prepared by heating and melting the material to be dispersed, and while in molten condition mixing it with vigorous stirring with a hot concentrated aqueous soap solution and continuing the stirring at a temperature above the melting point of the material until the dispersion of such material has been effected, whereupon the dispersion is allowed to cool. The dispersion consists of finely divided, congealed particles of the waterproofing material enveloped or protected by the soap dispersing solution, which prevents the coalescence of the particles into larger particles while the particles are in molten condition and after they have become congealed, so that when the dispersion is subsequently diluted in water there is very little tendency for the particles to separate or float out.

Another procedure for forming a substantially stable or non-separating dispersion may be as follows. The thermo-plastic material is added, with stirring, to a hot aqueous solution of soap-forming constituents, e. g., a fatty acid or fatty acid glyceride, and a solution of a suitable saponifying agent, such as caustic soda, and the mass is stirred and maintained at a temperature above the melting point of the thermoplastic material until the dispersion has been effected, whereupon the dispersion is allowed to cool. The cool dispersion comprises finely divided particles of congealed thermoplastic material, protected or filmed by the soap, formed from the reaction of the soap-forming constituents, which functions to prevent the formation of large agglomerates, during the dispersing procedure and after the dispersion has been effected, and produces a substantially stable, non-separating dispersion.

This dispersion is essentially similar to the

dispersion produced by adding a molten thermoplastic material to a previously formed soap. When waterproofing materials fluid at atmospheric temperature, such as mineral oils, are employed, no heating would of course be necessary.

I have found that when a soap dispersion of waterproofing material such as described, containing a large proportion of unsaponified waterproofing material, is incorporated into pulp in the beater engine and precipitated with aluminum sulphate, alum, or other coagulating agents, a considerable proportion of the dispersed material remains behind as fine particles, and is not brought down and fixed on the stock together with the precipitated aluminum soap. In other words, the factor or retentivity of the dispersed material by the pulp is not optimum, a substantial percentage of such material being subsequently lost in the water removed during subsequent paper-forming operation, without performing a sizing or waterproofing function. For example, in employing a paraffin soap dispersion for sizing pulp which contains 1.5 to 5 parts of paraffin to about 10 parts of rosin size, it is found that it is uneconomical to incorporate more than 5% of paraffin into the pulp, because of the high loss of paraffin which results, due to separation of the paraffin after the coagulation of the dispersing agent. Moreover, it is uneconomical to operate with a dispersion containing a high percentage of paraffin or other like waterproofing material based on the weight of soap-dispersing agent, because of the consequent low retentivity resulting if high percentages of paraffin are employed, inasmuch as the soap serves the function of fixing the dispersed particles on the pulp.

In certain cases, however, it is desirable to incorporate higher than 5% paraffin or other waterproofing material into the stock so as to produce a paper of high waterproofing quality, and to incorporate such waterproofing material without the introduction of an excessive quantity of aluminum resinate or other insoluble soaps, which are inferior as waterproofing or sizing agents to paraffin or other like unsaponified thermoplastic or waterproofing materials.

I have discovered that if the precipitation of an aqueous paraffin-soap dispersion or like dispersions of waterproofing ma-

terial is effected in the presence of a soluble precipitable agent capable of uniting with aluminum sulphate or alum and forming a sufficient quantity of a voluminous or flocculent precipitate, the dispersed, unsaponified particles of waterproofing material are brought down substantially in entirety, and together with the aluminum soap are fixed on the fibers of the pulp, thus resulting in a high factor of retentivity and hence a very low loss of such material in the water removed during subsequent paper-forming operation. Large percentages of paraffin or other waterproofing material may thus be economically employed for waterproofing paper.

The following example sets forth one method of procedure which may be employed in the preparation of a paraffin-soap dispersion which has been found to yield excellent results in sizing pulp. About 100 pounds of commercial rosin size (consisting of 40 parts of dry rosin size and 60 parts of water) is heated to about 120° F. A heated mixture of silicate of soda and paraffin is formed by adding 40 parts of silicate of soda (60° Baumé) to 40 parts of paraffin and, while stirring, heating the mixture above the melting point of the paraffin (say, 130° F.). To the heated solution of rosin size is added, with vigorous stirring, the heated mixture of silicate of soda and paraffin, and the mixed mass is stirred and maintained at a temperature of about 130° F. for about 15 to 20 minutes, whereupon the dispersion of the paraffin is completed. The dispersion is of a heavy, creamy consistency, and consists of fine, discrete particles of paraffin, enveloped by films of sodium resinate which serve to prevent the coalescence of the particles and to maintain the dispersion in substantially stable or non-separating form, so that upon dilution with water there is little tendency for the particles to separate or float out. The dispersion is preferably cooled prior to addition to the stock to be sized in the beater engine, so as to prevent a tendency to excessive foaming.

Another example of procedure for the preparation of a paraffin-soap dispersion may be about as follows. About 100 parts of commercial rosin size are added, with stirring, to about 40 pounds of paraffin, and are cooked together at a temperature of about 130° F. for about 30 minutes, whereupon the paraffin becomes dispersed as fine particles in the soap solution and yields a substantially stable, non-separating dispersion. About 40 parts of sodium silicate (60° Baumé) is mixed into the dispersion and, preferably after allowing the mixture to cool, it may be incorporated into the stock to be sized in the beater engine.

I prefer to employ the procedure described in the first example, because the dis-

persed particles appear to be in much finer condition and there is less tendency for the particles to agglomerate and separate out when diluted with water. This may be due to the fact that the dispersion is not only produced by the size (sodium resinate), but also by the sodium silicate, which itself is a very effective dispersing agent. Consequently, the combined dispersive effect is greater than by the use of the rosin size or other soap alone.

The paraffin soap dispersion thus produced may be added to the pulp in the beater engine prior to its manufacture into paper. About 180 pounds of dispersion may be added, for example, to size about 1000 pounds of sulphite pulp, which may be formed into paper of a highly water-resistant and non-absorbent character, suitable for a great variety of uses. The addition of the dispersion preferably takes place during the last stages or after the completion of the beating operation, so as to avoid a tendency to excessive foaming. After the dispersion is incorporated into the pulp, the rosin and sodium silicate are simultaneously precipitated by the addition of aluminum sulphate or alum to the beater, about 150 to 200 pounds of alum being sufficient to ensure the precipitation of all the sodium silicate and rosin. The aluminum silicate comes down as a voluminous or flocculent precipitate, which, aided by the aluminum resinate soap, carries along therewith, or "pulls down" substantially all the finely dispersed particles of paraffin, and fixes them on the fibers of the pulp. The factor of retentivity of dispersed paraffin thus fixed on the stock is high and consequently large percentages of dispersed unsaponified material may economically be incorporated into pulp to produce paper having high waterproofing characteristics.

In the drying and calendering operations, the dispersed particles of paraffin are heated above their melting point, causing them to flux together with the aluminum resinate, and resulting in the melting and coalescence of the sizing particles throughout the paper. The precipitated aluminum silicate serves as an admirable filler or loading material, and adds bulk and opaqueness to the paper. The amount of sodium silicate added to the pulp should be regulated with the percentage of paraffin which is to be "pulled down" or precipitated on the pulp, and consequently if the percentage of paraffin is varied, the percentage of sodium silicate may also be correspondingly varied, but in any event, sufficient sodium silicate should be added to ensure a substantially complete retention of the paraffin.

While I have described certain specific examples of procedure which have been found to yield desired results in papers suit-

able for certain uses, it is obvious that I 5  
may modify the percentages of the various  
agents as desired, depending upon the char-  
acter of the paper which it is desired to pro-  
duce and the uses to which it is to be put.  
The percentage of paraffin in the dispersion,  
based on rosin or other soap, may be main-  
tained as high as is consistent with the pro-  
duction of a substantially stable or non-

10 separating dispersion, but any other suitable  
proportion of paraffin to rosin may be used,  
if desired. I may also replace a portion or  
all of the paraffin by other waxes, such as  
15 Montan, carnauba, Japan, candelilla, or  
other unsaponifiable or difficulty saponifi-  
able waterproofing material, and a portion  
or all of the rosin, by other soaps, such as  
sodium oleate, sodium palmitate, sodium  
20 stearate, and the like.

25 It is also possible to change or modify the  
procedure from that described in these  
specific examples. Thus I may incorporate  
the soap-paraffin dispersion into the stock  
in the beater engine, and add sodium silicate  
30 separately thereto; or I may first add the  
aluminum sulphate or alum to the stock and  
subsequently incorporate the paraffin-soap  
dispersion and sodium silicate, but the pro-  
cedure set forth in the examples given has  
35 generally been found to be more expedient.  
Other sizing and filling agents may also be  
used together with those agents mentioned.  
The dispersion may also be successfully em-  
ployed in the sizing of various pulp  
40 furnishes.

45 In carrying on experimentation connected  
with the discoveries disclosed herein, I found  
that I may substitute caustic soda or caustic  
lime, or equivalent alkaline compounds, for  
the sodium silicate, and produce a precipi-  
tate of aluminum hydrate which also per-  
forms the function of carrying down there-  
with the dispersed particles of unsaponified  
waterproofing material. The results pro-  
duced thereby, however, are inferior to those  
50 obtained by the use of sodium silicate, and  
the retentivity of dispersed particles by the  
stock is lower; also a larger quantity of  
alum must be used.

55 This is doubtless due to the fact that the  
aluminum hydrate is of much lower bulk  
than the aluminum silicate precipitate, and  
consequently does not carry the dispersed  
particles down as efficiently. The essential

factor appears to consist in the precipitation 55  
of a voluminous or flocculent precipitate,  
which carries down therewith the fine par-  
ticles of unsaponified dispersed thermo-  
plastic material and fixes them on the fibers  
of the pulp together with the insoluble soap 60  
formed from the soluble soap which serves  
as the dispersing agent.

I claim:

1. A process of sizing paper, which com-  
prises incorporating into pulp prior to its 65  
formation into paper, an aqueous soap dis-  
persion of unsaponified waterproofing ma-  
terial, together with a substantial quantity  
of sodium silicate, and adding sufficient  
aluminum sulphate to precipitate the soap 70  
and sodium silicate, thereby forming a vol-  
uminous precipitate of aluminum silicate  
carrying down and fixing substantially all  
the dispersed material on the pulp.

2. A process of sizing paper, which com-  
prises adding to pulp prior to its formation 75  
into paper, an aqueous soap-sodium-silicate  
dispersion of unsaponified waterproofing  
material, and adding sufficient aluminum  
sulphate to precipitate the soap and silicate,  
80 thereby forming a voluminous precipitate of  
the aluminum silicate carrying down and fix-  
ing substantially all the dispersed material  
on the pulp.

3. A process of waterproofing paper, 85  
which comprises incorporating into pulp  
prior to its formation into paper, an aqueous  
sodium resinate dispersion of unsaponified  
waterproofing material, together with a sub-  
stantial quantity of sodium silicate, and add-  
ing sufficient aluminum sulphate to precipi-  
tate the sodium silicate, thereby forming a 90  
voluminous precipitate of aluminum silicate  
carrying down and fixing substantially all  
the dispersed material on the pulp. 95

4. A process which comprises incorporat-  
ing into paper pulp an aqueous sodium resi-  
nate dispersion of thermoplastic water-  
proofing material together with sodium sili-  
cate, adding alum in sufficient quantity 100  
to precipitate substantially all the resinate  
and silicate, running the pulp out on a paper  
machine, and fusing the thermoplastic ma-  
terial in the paper.

In testimony whereof I have affixed my 105  
signature.

ALBERT L. CLAPP.